

3,822,136

## SILVER HALIDE LIGHT-SENSITIVE SUPERSENSITIZED MATERIALS

Kaichiro Sakazume, Shui Sato, Noboru Fujimori, and Eiichi Sakamoto, Hanno, and Kiyomitsu Mine, Tokyo, Japan, assignors to Konishiroku Photo Industry Co., Ltd., Tokyo, Japan  
No Drawing. Filed Sept. 20, 1972, Ser. No. 290,512  
Claims priority, application Japan, Sept. 27, 1971,

46/74,631

Int. Cl. G03c 1/14

U.S. Cl. 96—126

5 Claims

### ABSTRACT OF THE DISCLOSURE

This invention provides a light-sensitive material of the silver halide type having high speed green sensitivity and being highly supersensitized to green light, which comprises a silver halide photographic emulsion and a specific combination of at least one compound expressed by following formula (I)



with at least one compound expressed by following formula (II)



This light-sensitive material can be applied to not only black-and-white photography but also color photography, and is excellent over conventional supersensitized light-sensitive emulsions in spectral sensitivity, good storability, high color reproducibility with less color contamination, and other photographic characteristics.

This invention relates to a light-sensitive material of the silver halide type exhibiting an excellent supersensitizing effect. More particularly, the invention relates to a photographic material of the silver halide type which has a high green sensitivity and is highly supersensitized to light of the green portion of the spectrum.

The inherent sensitivity of silver halide emulsions is confined to short wavelength regions, namely ultraviolet and blue regions of the spectrum. It is known that the sensitivity of silver halide emulsions can be extended effectively by the use of certain dyes of the cyanine or merocyanine type. It is also known that when, in combination with such sensitizing dye, a certain other sensitizing dye or organic compound is incorporated into a silver halide emulsion, it is possible to impart to the emulsion a sensitivity higher than the sum of the individual effects of these sensitizing materials. Such effect is called "supersensitizing effect."

In case such supersensitizing method is actually applied to silver halide emulsions in the photographic industry, it is desired that in addition to attainment of good spectral sensitizing effect, the following requirements will be satisfied:

- (1) The spectral sensitization can be attained properly in the intended portion of the spectrum.
- (2) The sensitizing material to be added does not cause such a reaction with other photographic additives as will result in bad influences to the quality of the resulting photographic material, and photographic charac-

teristics of a photosensitive film or paper can be retained during storage stably.

(3) Fog or dye contamination is not observed on a photographic film or paper after development.

5 When the supersensitizing method is applied to green-sensitized emulsions for use in preparing light-sensitive materials for color photography, it is especially important that these requirements will be satisfied. More specifically, it is desired that the emulsions have a sensitized spectrum portion optimum to exhibit a good color reproducibility as materials for color photography and have a green sensitivity of a high speed with less color contamination. Although various combinations of sensitizing dyes have been heretofore proposed to provide supersensitized silver halide emulsions, most of them fail to satisfy the above requirements sufficiently.

10 It is therefore a primary object of this invention to provide a highly supersensitized silver-halide light-sensitive material which will meet all of the above requirements sufficiently.

15 Another object of this invention is to provide a combination of sensitizing dyes which gives such excellent supersensitized photographic material of the silver halide type.

20 25 Still another object of this invention is to give a green sensitivity of a high speed to a silver halide emulsion.

Other objects and advantages of this invention will be apparent from the description given hereinbelow.

25 As a result of extensive research works we have now 30 found that the above objects and advantages can be attained by incorporating in a silver halide emulsion at least one member selected from compounds expressed by the following general formula (I)



35 wherein R<sub>1</sub> and R<sub>3</sub> stand for a lower alkyl group having 1 to 3 carbon atoms or a sulfoalkyl group; R<sub>2</sub> designates a hydrogen atom or a lower alkyl group having 1 to 3 carbon atoms; Y<sub>1</sub>, Y<sub>2</sub>, Y<sub>3</sub>, Y<sub>4</sub>, Y<sub>5</sub> and Y<sub>6</sub> stand for a hydrogen or halogen atom, a lower alkyl group having 1 to 3 carbon atoms, a lower alkoxy group having 1 to 3 carbon atoms or phenyl group, or they may be atomic groups bonded together to form a naphthoxazole nucleus; X<sup>(-)</sup> indicates an acid anion; and n is 0 to 1, and at least one member selected from compounds expressed by the following general formula (II)



45 55 wherein R<sub>4</sub> is a lower alkyl group having 1 to 3 carbon atoms, a hydroxyalkyl group, a carboxyalkyl group or a sulfoalkyl group; Z is an atomic group necessary for forming an oxazole, benzoxazole, naphthoxazole, benzimidazole, thiazoline, thiazole, benzothiazole, naphthothiazole, indolene or pyrrolidine nucleus which may be substituted by a halogen atom, a lower alkyl group having 1 to 3 carbon atoms, a lower alkoxy group having 1 to 3 carbon atoms, a phenyl group or a hydroxyl group; and Q is an atomic group necessary for forming a rhodanine, thiohydantoin or 2-thioxazolidinedione nucleus which may be substituted by a hydroxyalkyl group, an alkoxyalkyl group, a carboxyalkyl group, a sulfoalkyl group, a lower alkyl group having 1 to 3 carbon atoms, a phenyl group or a halogen-substituted phenyl group.

Thus, in accordance with this invention there is provided a photographic material of the silver halide type which comprises a silver halide photographic emulsion and, incorporated therein, a combination of at least one member selected from compounds expressed by the above general formula (I) with at least one member selected from compounds expressed by the above general formula (II).

In the photographic material of this invention comprising a combination of the above-mentioned specific sensitizing compounds expressed by the general formulae (I) and (II), it is possible to attain excellent spectral supersensitization in either or both of the shorter wavelength portion and longer wavelength portion of the green region of the spectrum. Furthermore, the photosensitive material of this invention makes it possible to photograph an ob-

ject having a specific reflective spectrum or to effect the photographing under a specific light source.

Further, the sensitizing compounds of the above formulae (I) and (II) do not cause such a reaction with additives contained in photographic emulsions as will affect 5 badly these additives or resulting photographic materials. When a silver halide emulsion comprising the sensitizing compounds of this invention is coated on a substrate film or paper, there is obtained a photographic material in 10 which no color contamination is left behind after development and which is excellent in spectral supersensitization.

Compounds expressed by the above general formulae (I) and (II) will now be illustrated, but the scope of this invention is not limited by such illustration.

15 Typical instances of compounds expressed by the general formula (I) are as follows:

| Compound No. | Structural formula | Maximum absorption wavelength<br>( $\mu$ ) in<br>methanol |
|--------------|--------------------|-----------------------------------------------------------|
| (1)-----     |                    | 496                                                       |
| (2)-----     |                    | 498                                                       |
| (3)-----     |                    | 503                                                       |
| (4)-----     |                    | 503                                                       |
| (5)-----     |                    | 518                                                       |
| (6)-----     |                    | 507                                                       |
| (7)-----     |                    | 524                                                       |
| (8)-----     |                    | 487                                                       |

As typical instances of compounds expressed by the above general formula (II), the following compounds may be mentioned:

| Compound No. | Structural formula | Maximum absorption wavelength (m $\mu$ ) in methanol |
|--------------|--------------------|------------------------------------------------------|
| (9)          |                    | 493                                                  |
| 10)          |                    | 488                                                  |
| (11)         |                    | 488                                                  |
| (12)         |                    | 470                                                  |
| (13)         |                    | 486                                                  |
| (14)         |                    | 516                                                  |
| (15)         |                    | 480                                                  |
| (16)         |                    | 480                                                  |

TABLE—Continued

| Compound No. | Structural formula | Maximum absorption wavelength (m $\mu$ ) in methanol |
|--------------|--------------------|------------------------------------------------------|
| (17).....    |                    | 480                                                  |
| (18).....    |                    | 480                                                  |
| (19).....    |                    | 496                                                  |
| (20).....    |                    | 488                                                  |

These compounds may be synthesized by methods disclosed in French Pat. 1,108,788 Specification, Japanese Patent Publication 13,821/68, etc.

Silver halide light-sensitive materials of this invention, which have excellent photographic characteristics such as mentioned above, may be effectively applied to not only high speed black-and-white emulsion but also color light-sensitive photography. According to this invention, it is also possible to provide coloring dye-containing light-sensitive materials for color photography by the silver dye bleach method.

In silver halide light-sensitive materials of this invention, the distribution of the maximum sensitization wavelength may be varied depending upon the kinds of compounds of the general formulae (I) and (II) and the mixing ratio of them.

These compounds are usually incorporated into a silver halide emulsion in the state dissolved in water or an organic solvent such as methanol and ethanol, or a mixture thereof. They may be added to the silver halide emulsion at any time during the emulsion preparation process, but it is generally preferred that the addition is effected just after the second-ripening step. The amounts added of the compounds of the general formulae (I) and (II) vary depending upon the kind of the silver halide emulsion, but in general it is preferred that they are added in such amounts that the sum of them is 1 to 500 mg. per mole of the silver halide. It is also preferred that the mixing ratio of both the compounds is within a range of from 1:10 to 10:1.

Emulsions of any of silver chloride, silver chloride-bromide, silver bromide, silver iodide-bromide and silver iodide-chloride-bromide may be used as the silver halide emulsion in this invention. It is permissible that these emulsions may be sensitized by noble metal sensitizers,

sulfur sensitizers, reduction sensitizers or sensitizers of the polyalkylene oxide type. Further, these emulsions may further comprise additives such as stabilizers, surfactants and hardening agents.

45 This invention will now be illustrated by reference to Examples but it is not at all limited by these Examples.

#### Example 1

50 A high speed emulsion of the silver iodide-bromide type containing 3 mole percent of silver iodide was prepared by effecting the second-ripening by the gold sensitizing and sulfur sensitizing methods. Compounds of formulae (I) and (II) were added to the emulsion individually or 55 in combination as indicated in Table 1 given below. Each compound was incorporated in the form of a 0.1% methanol solution.

55 Each emulsion was maintained at about 40° C. for 20 minutes to stabilize the spectral sensitivity, and then it was uniformly coated on a cellulose triacetate film substrate and dried to obtain a sample.

60 Each sample was exposed to day-light of 160 luxes (5400° K.) with use of a sensitometer (model KS-1 manufactured by Konishiroku Photo. Ind. Ltd.) covered 65 with a green filter having a maximum percent transmission at 525 m $\mu$ , and then it was developed with a liquid developer having the following composition:

|                                      | G.               |
|--------------------------------------|------------------|
| N-methyl-p-aminophenol sulfate ..... | 3.0              |
| Anhydrous sodium sulfite .....       | 50.0             |
| Hydroquinone .....                   | 6.0              |
| Sodium carbonate .....               | 29.5             |
| Potassium bromide .....              | 1.0              |
| Water .....                          | Balance          |
|                                      | Total, 2 liters. |

The development was conducted at 20° C. for 5 minutes. Then fixing and water-washing treatments were carried out according to customary methods. The speed of green sensitivity and fog were determined with respect to each sample to obtain results shown in Table 1, in which the value of the speed of green sensitivity is expressed in terms of a relative speed calculated on the assumption that the speed of green sensitivity attained by single use of compound (2) corresponds to a relative speed of 100. In Table 1, compound numbers correspond with those given hereinabove when compounds of formulae (I) and (II) being illustrated.

Each emulsion was immediately coated on a polyethylene terephthalate film substrate and dried to obtain an as-coated sample. Then, the as-coated sample was allowed to stand still at 50° C. for 3 days in a relative humidity of 80% to obtain a preserved sample for testing the storability under high temperature and high humidity conditions.

These samples were exposed and developed in the same manner as in Example 1 and the sensimetry was conducted to determine the speed of green sensitivity. Further, the spectral supersensitivity to 530-540 m $\mu$ , which is indispensable for faithful reproduction of a human image,

TABLE 1

| Sample number | Compound of Formula (I) |                           | Compound of Formula (II) |                           | Relative speed of green sensitivity | Maximum sensitivity wavelength (m $\mu$ ) |
|---------------|-------------------------|---------------------------|--------------------------|---------------------------|-------------------------------------|-------------------------------------------|
|               | Compound number         | Amount added <sup>1</sup> | Compound number          | Amount added <sup>1</sup> |                                     |                                           |
| 1             | (2)                     | 180                       |                          |                           | 100                                 | 552                                       |
| 2             |                         |                           | (10)                     | 180                       | 85                                  | 548                                       |
| 3             |                         |                           | (12)                     | 180                       | 72                                  | 530                                       |
| 4             | (2)                     | 120                       | (10)                     | 60                        | 170                                 | 550                                       |
| 5             | (2)                     | 90                        | (12)                     | 60                        | 165                                 | 550                                       |
| 6             | (5)                     | 180                       |                          |                           | 96                                  | 573                                       |
| 7             |                         |                           | (14)                     | 180                       | 80                                  | 570                                       |
| 8             | (5)                     | 120                       | (14)                     | 60                        | 171                                 | 570                                       |
| 9             | (5)                     | 120                       | (12)                     | 30                        | 153                                 | 570                                       |
| 10            | (6)                     | 180                       |                          |                           | 101                                 | 545                                       |
| 11            |                         |                           | (19)                     | 180                       | 88                                  | 550                                       |
| 12            |                         |                           | (9)                      | 180                       | 90                                  | 550                                       |
| 13            | (6)                     | 120                       | (19)                     | 60                        | 163                                 | 543                                       |
| 14            | (6)                     | 90                        | (9)                      | 60                        | 160                                 | 543                                       |

<sup>1</sup> Mg. per mole of silver halide.

From the results shown in Table 1, it is apparent that when compounds of general formulae (I) and (II) are employed in combination, the green sensitivity is highly improved over that attained by their individual use.

### Example 2

Compounds of general formulae (I) and (II) were added in a combination, as illustrated in Table 2, to a

30 was measured with use of an interference filter. In this measurement, the preserved sample was used. Results are shown in Table 2, in which the value of the speed of green sensitivity is expressed in terms of a relative speed calculated on an assumption that the speed of green sensitivity of the as-coated sample of the comparative emulsion corresponds to a relative speed of 100.

TABLE 2

| Sample number | Compound of Formula (I) |                           | Compound of Formula (II) |                           | Relative speed of green sensitivity | 530-540 m $\mu$ |
|---------------|-------------------------|---------------------------|--------------------------|---------------------------|-------------------------------------|-----------------|
|               | Compound Number         | Amount added <sup>1</sup> | Compound Number          | Amount added <sup>1</sup> |                                     |                 |
| 15            |                         |                           | (2)                      | 120                       | 60                                  | 165             |
| 16            |                         |                           | (5)                      | 120                       | 90                                  | 155             |
| 17            |                         |                           | (8)                      | 120                       | 60                                  | 160             |
| 18            | <sup>2</sup> (A)        | 90                        | <sup>2</sup> (B)         | 90                        | 100                                 | 85              |

<sup>1</sup> Mg. per mole of silver halide.

<sup>2</sup> Comparative.

high speed silver iodide/bromide emulsion similar to that used in Example 1. After the after-ripening, a suitable amount of 4-hydroxy-6-methyl-1,3,3a,7-tetrazaindene was added to the emulsion as an antifoggant to form a green-sensitive emulsion. As a comparative sample of the conventional supersensitized green-sensitive emulsion, there was prepared an emulsion in the same manner as above by employing a combination of the following dyes (A) and (B) according to the teaching of U.S. Pat. 2,688,545 Specification:

Comparative Dye (A)



Comparative Dye (B)



50 From the results shown in Table 2, it will readily be understood that as compared with the comparative sample, the samples according to this invention exhibit excellent spectral sensitivity and have such excellent green-sensitive characteristics that the sensitivity is hardly changed on storage under severe conditions and the sensitivity to the spectral region of 530-540 m $\mu$ , which is essential for faithful reproduction of a human image, is extremely high.

### Example 3

60 A high speed emulsion of the silver iodide/bromide type for negative prints of color light-sensitive material containing 5 mole percent of silver iodide was gold-sensitized and sulfur-sensitized to effect the after-ripening, and anhydro - 5,5' - dichloro-3,3'-disulfopropyl-9-ethylthiocyaninehydroxide was added as a red-sensitizing dye in an amount of 150 mg. per mole of the silver halide. A cyan coupler formed by dissolving 4-chloro-1-hydroxy-2-n-octynaphthoic acid under heat into dibutyl phthalate and ethyl acetate and dispersing the solution into a gelatin solution with use of sodium alkylbenzenesulfonate was added to the emulsion. The pH of the emulsion was adjusted to 6.3, and the emulsion was coated uniformly on a cellulose triacetate film substrate, followed by drying. A thin gelatin layer was formed on the above emulsion coating. A high speed emulsion of the silver iodide/bromide type, similar to that employed in Example 1, was

11

incorporated with compounds of formulae (I) and (II) individually or in combination as indicated in Table 3 given below. In the same manner as described above with respect to formation of the cyan coupler, 1(3-carboxyphenyl)-3-(4-stearoylaminophenyl)-5-pyrazolone was dispersed and incorporated as a magenta coupler into the silver halide emulsion. After the pH was adjusted to 6.8, the emulsion was coated on the gelatin layer, followed by drying.

A yellow filter layer composed of colloidal silver was further coated on the above silver halide emulsion coating. Then, a yellow coupler formed by emulsifying and dispersing 2-dodecyloxybenzoyl acetoanilide in a gold-sensitized and sulfur-sensitized emulsion of the silver iodide/bromide type for negative film in the same manner as described above with respect to formation of the cyan coupler and magenta coupler, and the pH of the emulsion was adjusted to 6.8. The so formed yellow coupler emulsion was coated on the above yellow filter layer and dried to obtain a sample of a multi-layer light-sensitive material for color photography. The sample was exposed in the same manner as in Example 1 and developed at 22° C. for 10 minutes with use of a color developer of the following composition:

|                                                  |         |      |  |
|--------------------------------------------------|---------|------|--|
| N - ethyl - N-methanesulfoneamidoethyl-3-methyl- |         |      |  |
| aminoaniline sulfate                             | g       | 2.5  |  |
| Anhydrous sodium sulfite                         | g       | 2.0  |  |
| Benzyl alcohol                                   | cc      | 3.8  |  |
| Sodium hexametaphosphate                         | g       | 2.0  |  |
| Sodium carbonate (monohydrate)                   | g       | 50.0 |  |
| Potassium bromide                                | g       | 1.0  |  |
| Sodium hydroxide                                 | g       | 0.6  |  |
| Water                                            | Balance |      |  |
| Total, 1 liter.                                  |         |      |  |

After the development, the bleaching, fixing and water-washing treatments were carried out according to customary procedures. The color sensimetry was effected with respect to each sample to determine the speed of green sensitivity, fog (color contamination) and photographic gamma. Results are shown in Table 3, in which the value of the speed of green sensitivity is expressed in terms of the relative speed calculated on an assumption that the speed of green sensitivity attained by the single use of compound (6) corresponds to a relative speed of 100.

TABLE 3

| Sample number | Compound of Formula (I) |                           | Compound of Formula (II) |                           | Relative speed of green sensitivity | Fog (color contamination) | Photographic gamma |
|---------------|-------------------------|---------------------------|--------------------------|---------------------------|-------------------------------------|---------------------------|--------------------|
|               | Compound number         | Amount added <sup>1</sup> | Compound number          | Amount added <sup>1</sup> |                                     |                           |                    |
| 19            | (6)                     | 180                       |                          |                           | 100                                 | 0.07                      | 0.50               |
| 20            | (8)                     | 120                       | (12)                     | 60                        | 165                                 | 0.03                      | 0.55               |
| 21            | (3)                     | 120                       | (14)                     | 60                        | 160                                 | 0.03                      | 0.57               |
| 22            | (2)                     | 120                       | (18)                     | 60                        | 170                                 | 0.03                      | 0.60               |

<sup>1</sup> Mg. per mole of the silver halide.

From the results shown in Table 3, it will readily be understood that samples formed according to this invention exhibit excellent spectral sensitization, and with improvement in the photographic gamma, clear images of less color contamination can be obtained after the development treatment.

What we claim is:

What we claim is:

1. A light-sensitive material of the silver halide type which comprises a silver halide emulsion and, incorporated therein, a combination of at least one member selected from compounds expressed by the following general formula (I)



12

wherein  $R_1$  and  $R_3$  stand for a lower alkyl group having 1 to 3 carbon atoms or a sulfoalkyl group;  $R_2$  designates a hydrogen atom or a lower alkyl group having 1 to 3 carbon atoms;  $Y_1$ ,  $Y_2$ ,  $Y_3$ ,  $Y_4$ ,  $Y_5$  and  $Y_6$  stand for a hydrogen or halogen atom, a lower alkyl group having 1 to 3 carbon atoms, a lower alkoxy group having 1 to 3 carbon atoms or phenyl group, or they may be atomic groups bonded together to form a naphthoxazole nucleus;  $X^{(-)}$  indicates an acid anion; and  $n$  is 0 or 1, with at least one member selected from compounds expressed by the following general formula (II).



20 wherein  $R_4$  is a lower alkyl group having 1 to 3 carbon atoms, a hydroxylalkyl group, a carboxyalkyl group or a sulfoalkyl group; Z is an atomic group necessary for forming an oxazole, benzoxazole, naphthoxazole, benzimidazole, thiazoline, thiazole, benzothiazole, naphthothiazole, indolenine or pyrrolidine nucleus which may be substituted by a halogen atom, a lower alkyl group having 1 to 3 carbon atoms, a lower alkoxy group having 1 to 3 carbon atoms, a phenyl group or a hydroxy group, and Q is an atomic group necessary for forming a rhodanine, thiohydantoin or 2-thioxazolinedione nucleus which may be substituted by a hydroxylalkyl group, an alkoxyalkyl group, a carboxyalkyl group, a sulfoalkyl group, a lower alkyl group having 1 to 3 carbon atoms, a phenyl group or a halogen-substituted phenyl group.

35 2. A silver halide light-sensitive material set forth in claim 1 wherein the sum of amounts incorporated of the compounds of the above general formulae (I) and (II) is 1 to 500 mg. per mole of the silver halide contained in the gelatinous emulsion.

40 3. A silver halide light-sensitive material set forth in claim 1 wherein the ratio of the compound of the above general formula (I) to the compound of the above general formula (II) is within a range of from 10:1 to 1:10.

4. A silver halide light-sensitive material set forth in claim 1 wherein the silver halide is selected from silver

chloride, silver chloride/bromide, silver bromide, silver iodide/bromide and silver iodide/bromide/chloride.

5. A silver halide light-sensitive material according to claim 1 wherein the silver halide emulsion contains color coupling agents.

## References Cited

UNITED STATES PATENTS

- 3,671,260 6/1972 Oftedahl et al. ----- 96-126  
 3,711,288 1/1973 Sato et al. ----- 96-140

## FOREIGN PATENTS

- 625,446 6/1949 Great Britain ----- 96-126

200 21 227